

## UNITED STATES PATENT OFFICE.

ENEQUIQUE VINCKE, OF BARCELONA, SPAIN, ASSIGNOR TO MANUFACTURAS DE CORCHO S. A., OF BARCELONA, SPAIN, A LIMITED CORPORATION OF SPAIN.

## COMPOSITION CORK AND THE MANUFACTURE THEREOF.

No Drawing.

Application filed November 22, 1923. Serial No. 676,291.

This invention relates to improvements in the art of manufacturing composition cork in the form of thin sheets or webs and to the improved product resulting therefrom. The 5 object of the invention is to produce an improved sheet or web of composition cork of superior quality which may be used without splitting or skiving for such purposes as gaskets and other packings, bottle closures 10 and the like and in fact any purpose for which thin sheets of cork are desirable.

The physical properties of cork are such as to render it a highly desirable material for many industrial uses such as packings, heat 15 and sound insulation, floor coverings and the like, but in its natural state the size and shape of the pieces of cork bark and the varying quality thereof are such as to seriously limit its use. In view of these facts, cork has for 20 many years been made up into blocks, slabs, rods or heavy sheets, by assembling what is commercially termed granulated cork with or without a binder and subjecting the same to heat and pressure to compact the mass and 25 unite the particles one to another. The heating of cork particles to a sufficiently high temperature, for example, from 500° F. to 600° F., drives off moisture and partially volatilizes and otherwise liberates the inherent resinous 30 matter contained in the cork and causes at least part of the resinous matter to be so disposed in relation to the surfaces of the cork particles as to act as a binder when the particles are subjected to pressure to hold them one 35 to another and to protect the exposed surfaces of the particles so as to close and effectively seal the natural pores or cells and render the cork product substantially non-absorptive and less permeable than natural cork. 40 But whenever these blocks, slabs, rods or heavy sheets are cut, split or skived to form disks, thin sheets or other articles, as they commonly are to obtain pieces of usable dimensions, the particles of cork are divided by 45 the cutting knife so as to expose new surfaces which are not protected by the resinous matter and the product again becomes absorptive and more permeable. This is particularly true and particularly detrimental in the case 50 of thin sheets or disks wherein a single particle may be thus exposed on both sides of the sheet or disk.

It has long been known that when cork particles are subjected to a sufficiently high 55 degree of temperature to cause the inherent

cementitious matter to function as a binder, for example, to a temperature varying from 500 to 600° F., or even higher, the cork gives off various gases equaling many times its volume. If cork particles are so heated and 60 simuleaneously subjected to pressure the forces generated by the liberation of gases are tremendous and the gases should be permitted to escape at least in part. In the manufacture of composition cork in the form 65 of blocks, slabs, heavy sheets, rods and the like, moulds with loose fitting parts are commonly used so that the gases generated by the applied heat may pass through the relatively thick mass of cork to the crevices between the 70 mould parts and thereby escape. Heretofore the problem of disposing of the gases so generated has rendered it impossible, in so far as I am aware, to produce in a commercially satisfactory manner relatively thin 75 sheets or webs of composition cork under such conditions of temperature and pressure as will liberate the natural or inherent resinous matter contained in the cork and render the same effective as a binding and protective material. 80

It is an object of the present invention to produce thin moulded sheets of composition cork, that is, sheets moulded to usable thickness of about three-sixteenths of an inch or 85 less and not necessarily split or skived, and in which the resinous matter inherent in the cork has been rendered effective to bind the particles together and render the product relatively non-absorptive and impermeable. 90 Such sheets may even be as thin as four-thousandths of an inch.

In the practice of the present invention the cork is first subdivided into relatively small particles or obtained in that form, that is to 95 say, particles preferably having at least one dimension not exceeding the thickness of the finished sheet by more than the extent of compression to which the cork particles are to be subjected. For example, if the cork particles are to be compressed one-sixth, it is desirable that at least one dimension shall not be more than six times greater than the thickness of the finished sheet. Preferably the particles are selected so that at least one 100 dimension will be somewhat less than above stated in order that in the finished sheet the particles may more certainly partially overlap one another. The preferred form of cork particle used has a substantial surface area 105 110

in relation its thickness as for instance a substantially flat particle formed by shaving or chipping the natural cork.

In carrying out the invention a layer of 5 cork particles several times the thickness of the finished sheet is formed upon a suitable support so that the same may be subjected to the necessary heat and pressure. If desired, suitable cementitious material may be mixed 10 with the cork particles, but preferably the natural resinous matter contained in the cork itself is alone relied upon to cement the particles together. If it is desired to form a continuous web this layer of cork particles may 15 be introduced between cooperating endless conveyors which are urged toward each other by suitable pressure means or if separate sheets are to be formed the cork may be introduced between the platens of a suitable 20 press provided with means for heating and cooling the platens.

The volatile gases formed when the cork is subjected to heat are permitted to escape directly from the surface of the sheet or web 25 and preferably from the entire surface, as, for example, by interposing a piece of fine mesh wire cloth between the cork and the smooth surfaced platen of the press preferably on both sides of the cork. When the platens of 30 the press are brought together under sufficient pressure to compress the cork, for instance, to one-sixth or even to one-twentieth of its original volume, the cork will be pressed into the interstices of the metal cloth but on the 35 opposite side where the cloth comes in contact with the smooth surface of the platen, minute passages will be left open by which the gases generated when heat is applied can escape and be dissipated from the edges of 40 the press.

Preferably the cork particles are subjected to a temperature of approximately 575° F. while under pressure and for a time depending upon the thickness of the material. With 45 a thin gasket material of a thickness of about one-sixteenth of an inch, the heat and pressure will need to be maintained only for a very short time because the cork, due to the thinness of the sheet, will readily heat 50 through and the resinous matter will be partly volatilized and otherwise liberated so as to firmly cement one particle of cork to another and so dispose of the resinous matter in relation to the surface of the sheet as to 55 render the product more nearly impermeable than presently known products. The amount of pressure to which the cork particles are subjected may be varied within wide limits and will depend upon the quality, form and 60 condition of the cork particles, upon the extent to which it is desired to compress the cork relatively to its natural state and upon the character desired for the finished product and the use for which it is intended.

65 Preferably the cork is cooled while being

maintained under pressure, as by the introduction of a suitable heat exchange medium into the platens of the press when a platen press is used or by moving the conveyors to a cooling station if a continuous web is being 70 formed.

Thin sheeted cork produced in accordance with and embodying the present invention may be characterized by the perceptibly flattened appearance of the cork particles in the 75 finished sheet and the partial overlapping of adjacent particles. Such sheets will possess tensile strength to a high degree and will also be unusually flexible. Furthermore, the natural resins contained in the cork which are 80 partially liberated by the applied heat will be so disposed in the relation of the surfaces of the finished product as to render the finished sheet more nearly impermeable than natural cork or any of the presently known 85 forms of composition cork and the natural pores will be closed and effectively sealed. Inasmuch as cork sheets of the present invention may be produced in such thin sheets as are ordinarily required for gaskets and other 90 packings, bottle closures and the like, these various particles may be died out from the sheets without the splitting or skiving which has heretofore been necessary. The present 95 process also overcomes the difficulties of thoroughly heating through a substantially thick body of cork material in the manufacture of composition cork.

It is to be understood that the present invention is not limited to the precise method 100 of procedure or to the product described above for illustration but may be variously modified and embodied within the scope of the subjoined claims.

I claim as my invention:

1. The improvement in the art of manufacturing composition cork in relatively thin individually moulded sheets, which consists in subjecting a thin layer of cork particles to heat and pressure over a substantial area and 110 permitting the escape directly from the surface of the sheet of gases formed by the application of heat while maintaining the pressure thereon.

2. The improvement in the art of manufacturing composition cork in relatively thin individually moulded sheets not exceeding three-sixteenths of an inch in thickness, which consists in subjecting a thin layer of cork particles to heat and pressure over a substantial area and permitting the escape directly from the surface of the sheet of gases formed by the application of heat while maintaining the pressure thereon.

3. The improvement in the art of manufacturing composition cork in relatively thin individually moulded sheets, which consists in subjecting a thin layer of cork particles to heat and pressure over a substantial area, 125 permitting the escape directly from the sur- 130

face of the sheet of gases formed by the application of heat while maintaining the pressure thereon, and thereafter cooling said moulded sheet while maintaining the pressure thereon.

4. The improvement in the art of manufacturing composition cork in relatively thin individually moulded sheets, which consists in subjecting a thin layer of cork particles to 10 heat and pressure over a substantial area and permitting the escape directly from the entire surface of the sheet of gases formed by the application of heat while maintaining the pressure thereon.

15 5. The improvement in the art of manufacturing relatively thin individually sheeted composition cork which consists in subjecting a thin layer of cork particles to sufficient pressure over a substantial area to materially 20 compress the same, simultaneously subjecting said particles to sufficient heat to cause the same to be firmly united one to another and, while said heat and pressure is being maintained, permitting the gases formed by the 25 application of heat to escape from the surface of the cork.

6. The improvement in the art of manufacturing composition cork in relatively thin individually moulded sheets, which consists 30 in assembling a thin layer of cork particles adjacent a fine mesh wire cloth, and subjecting said particles while so maintained to the action of heat and pressure.

7. The improvement in the art of manufacturing composition cork in relatively thin 35 individually moulded sheets, which consists in forming a thin layer of cork particles between coextensive screens of fine mesh wire cloth, and subjecting the cork particles to heat and pressure while so maintained. 40

8. As an article of manufacture, an individually moulded sheet of composition cork not exceeding three-sixteenths of an inch in thickness and comprising a multiplicity of 45 cork particles united by heat and pressure, with permissible escape of gases.

9. As an article of manufacture, an individually moulded sheet of composition cork not exceeding three-sixteenths of an inch 50 in thickness and comprising a multiplicity of cork particles bound to one another solely by their inherent cementitious matter.

10. As an article of manufacture, an individually moulded sheet of cork comprising a multiplicity of adhering particles moulded 55 under heat and pressure with accompanying liberation of gases to a usable thickness not exceeding three-sixteenths of an inch and having its surfaces rendered substantially impermeable by the resinous matter inherent in 60 the cork.

In testimony whereof, I have signed my name to this specification this 21st day of November, 1923.

ENRIQUE VINCKE.